

# UNITED STATES PATENT OFFICE.

JAMES GUNN, OF PHILADELPHIA, PENNSYLVANIA.

## FUEL.

No. 920,734.

Specification of Letters Patent.

Patented May 4, 1909.

Application filed December 11, 1908. Serial No. 467,007.

*To all whom it may concern:*

Be it known that I, JAMES GUNN, a subject of the King of Great Britain, residing at Philadelphia, in the county of Philadelphia and State of Pennsylvania, have invented a certain new and useful Improvement in Fuel, of which the following is a specification.

My invention relates to a new and useful improvement in fuel, and has for its object to provide an exceedingly simple and effective device of this character whereby the waste of anthracite or bituminous coal may be used in place of coal that is usually employed in kitchen ranges, stoves, heaters and the like, and to this end it contemplates the production of briquets by molding the waste material and fixing it with a binding medium which produces a firm product that will not disintegrate from handling or moisture.

With these ends in view, this invention consists in the details of construction and combination of elements hereinafter set forth and then specifically designated by the claim.

In order that those skilled in the art to which this invention appertains may understand how to make and use the same, I will describe its construction in detail.

My improved fuel consists essentially of either anthracite or bituminous coal dust or fine coal cemented together with a mixture of common clay and tar water, which will bind the particles of coal together so that it will stand handling and which will not crumble to powder when ignited.

In carrying out my process, I take three parts of anthracite or bituminous coal dust, or buckwheat or rice coal, and mix with it one part of common clay which has been previously saturated with tar water. The tar water is made by boiling one-quarter of a pound of tar in one gallon of water.

In practice the clay is saturated with the tar water and the coal or coal dust mixed therewith and then pressed into brick or ball form and allowed to dry, the drying process taking about six hours at which time the briquets may be used and it is found that they give off a great amount of heat, last longer than coal and will burn to a powder.

The ball form burns freely for cooking purposes or heat, while the brick form may be used for blanketing or for keeping the fire in over night.

Having thus fully described my invention, what I claim as new and useful, is—

The herein described process of forming a fuel composition consisting in saturating one part of common clay with tar water formed by dissolving one-quarter of a pound of tar in one gallon of water and adding thereto three parts of carbonous material and allowing the complete mixture to dry, as specified.

In testimony whereof, I have hereunto affixed my signature in the presence of two subscribing witnesses.

JAMES GUNN.

Witnesses:

JOHN MCKEE,  
ROBERT R. P. BRADFORD.